

## UNITED STATES PATENT OFFICE.

PHILIP MAGNUS, OF LEICHHARDT, NEAR SYDNEY, NEW SOUTH WALES, AUSTRALIA.

## MANUFACTURE OF ARTIFICIAL LEATHER.

No Drawing. Application filed February 12, 1926, Serial No 87,978, and in Australia March 2, 1925.

This invention relates to an improved process for the manufacture of artificial leather and to a material resulting therefrom.

5 In the carrying out of the process waste or scrap leather is utilized. Such leather is preferably first sieved or otherwise suitably treated for the purpose of separating therefrom grit or dirt or other extraneous matter.

10 The cleaned scrap or waste leather is then treated in a compounded mixture composed of the following ingredients:—glue, glycerine, boiled linseed oil, carbolic oil, ammonium bichromate and calcium chloride. Said treatment consists in adding to such mixture whilst it is being heated or boiled a sufficiency of the scrap or waste leather. Usually it will be found that to said mixture a proportion of approximately 25% of scrap or waste leather should be added during the heating or boiling operation. Before the scrap or waste leather is added to the mixture the latter is heated or boiled 15 until the whole of the ingredients thereof have become thoroughly incorporated.

20 When the ingredients of the compound consisting of the said liquid mixture with the waste or scrap leather are thoroughly blended the mass is placed in suitable moulds where it is subjected to appropriate pressure, say a pressure of from one quarter to one ton per square inch.

25 As one example of the liquid mixture the following ingredients in the following approximate proportions may be used:—

|                     | Per cent. |
|---------------------|-----------|
| Glue                | 70        |
| Glycerine           | 12½       |
| Boiled linseed oil  | 10        |
| Carbolic oil        | 2½        |
| Ammonium bichromate | 2½        |
| Calcium chloride    | 2½        |

45 Artificial leather in accordance with the invention may be used for the manufacture of boot or shoe heels and soles and other

articles. Such leather has been found to be less brittle; to have more waterproofing qualities; and to be easier of working than ordinary leather, whilst its cost of production and the manufacture of articles therefrom are economical.

50 In case of necessity any scrap or waste leather of a size too large for treatment as above described may previously be reduced in size to fit it for use in accordance with the process herein described. Glue is employed as an adhesive or binder; glycerine prevents the molded mass from becoming brittle; 55 ammonium bichromate renders the leather compound waterproof and insoluble in water; while the calcium chloride prevents the glue from cracking. Any substances other than carbolic oil can be utilized in 60 the liquid compound, such oil having for its object to avoid putrefaction of the artificial leather. Similarly, for boiled linseed oil any other suitable oil may be substituted; the said oil is added to the liquid compound to ensure the strength and drying 65 qualities of the artificial leather. In the appended claims the terms carbolic oil and boiled linseed oil are to be read to include any oils suitable for the purposes herein 70 described for which carbolic oil and boiled linseed oil are used in the liquid compound to which the scrap leather is added.

75 What I claim as my invention and desire to secure by Letters Patent is:—

80 1. An artificial leather consisting of cleaned scrap leather incorporated in a mixture of glue, glycerine, boiled linseed oil, carbolic oil, ammonium bichromate and calcium chloride.

85 2. An artificial leather consisting of cleaned scrap leather incorporated in a mixture of glue 70%; glycerine 12½%; boiled linseed oil 10%; carbolic oil 2½%; ammonium bichromate 2½% and calcium 90 chloride 2½%.

Artificial leather in accordance with the invention may be used for the manufacture of boot or shoe heels and soles and other

In testimony whereof I affix my signature.

PHILIP MAGNUS.